

Patented June 2, 1925.

1,540,424

# UNITED STATES PATENT OFFICE.

WALTER PHILIP REGESTEIN, OF WILMINGTON, DELAWARE, ASSIGNOR TO E. I. DU PONT DE NEMOURS & COMPANY, OF WILMINGTON, DELAWARE, A CORPORATION OF DELAWARE.

## METHOD OF PRODUCING NITROCELLULOSE EXPLOSIVES.

No Drawing.

Application filed July 17, 1919. Serial No. 311,512.

To all whom it may concern:

Be it known that I, WALTER PHILIP REGESTEIN, a citizen of the United States, and a resident of Wilmington, in the county of 5 New Castle and State of Delaware, have invented a certain new and useful Method of Producing Nitrocellulose Explosives, of which the following is a specification.

My invention relates to methods of producing nitrocellulose explosives and has more particular relation to the art of increasing the porosity of dense nitrocellulose powders by incorporating a soluble solid in the nitrocellulose and ultimately dissolving 10 out the solid, thereby to leave the nitrocellulose porous, and, hence, fast burning and desirable for use in practice ammunition, and in small calibre sporting rifles, pistols and revolvers. 15 Various methods involving this general feature have heretofore been proposed and the practice of incorporating a soluble solid in nitrocellulose, and its ultimate removal, is well known. For example, specific 20 methods have been proposed for the use of sugar, saltpetre or other suitable salts, of barium nitrate and of sodium nitrate.

The present invention has not to do, therefore, merely with this well known 25 practice of using a soluble solid, but relates more particularly to a method which, by its various features, adapts this practice to satisfactory and economical commercial use.

An object of the present invention is to 30 provide a method, in the aforesaid art, whereby complications are avoided, a superior product produced, and the solid body and the solvent for the nitrocellulose conveniently removed and recovered from the 35 product.

To this end, and also to improve generally upon methods of the character indicated, my invention consists in the following 40 matters hereinafter described and claimed.

In general, in proceeding according to 45 the present invention, in the preferable manner, I use a mixture of nitrocellulose having certain of its elements soluble in, and certain other of its elements not soluble in, the solvent used for the colloiding: I perform the colloiding of this mixture by treating it with a solution in which (as just indicated) all elements of the mixture are not

soluble, and which solvent can be ultimately removed by the extracting agent used to remove the solid body that is used for obtaining porosity, and simultaneously with the colloiding I add the said solid body and incorporate it with the nitrocellulose; I then form the colloid into grains by pressing 50 through a die of say about .05 inch in diameter and cutting the strings, say 100 to the inch; I then discharge the grains directly into a solvent which is a solvent not only for the solvent used for the nitrocellulose 55 but also for the solid body, thus removing both the solid body and the solvent for the nitrocellulose at the same time, and treat a sufficient time, and under such conditions as to remove both; I then drain and dry; and 60 then I cool, expose to absorb moisture, and perform the graphiting in the usual manner.

Thus, I provide a process which not only gives a product of superior porosity but also 65 can be successively and economically carried out commercially. The incorporation of the solid body simultaneously with the colloiding and the use of a mixture of nitrocellulose all elements of which are not soluble in 70 the solvent used for colloiding—as distinguished from the use of a solvent which is capable of dissolving all the nitrocellulose but is only used sufficiently to partially dissolve the nitrocellulose—gives a particularly 75 satisfactory product; and use of such a solid body, and such a solvent for the nitrocellulose, that both body and solvent can be removed simultaneously with a single solvent 80 gives a method well adapted for economical use commercially.

Preferably I use a mixture of nitrocellulose part of which is, and part of which is not, soluble in a mixture of ethyl ether and ethyl alcohol, and various proportions of 85 soluble to insoluble nitrocellulose may be used depending upon the powder desired, about 30 to 40% of soluble and 70 to 60% of insoluble being generally satisfactory. And preferably also, I use for the solid 90 body from 10 to 100 parts of certain salts such as potassium nitrate, sodium nitrate or sodium sulphate (preferably anhydrous) that are soluble in water,—the ethyl ether and ethyl alcohol being also soluble in 100 water—and can be extracted from the gran-

ulated powder by the use of hot water of suitable temperature for a suitable length of time.

The salts which I mention are examples 5 of solids which are without injurious action on the stability of the powder grain and can be substantially wholly extracted from the powder grains by treatment with the solvent for the solvent of the nitrocellulose and of 10 the solid body. For example, with these salts even when 100 parts of salt are incorporated in 100 parts of nitrocellulose the amount of salts not extracted is less than 1.5%. But, of course, other bodies fulfilling the desired 15 conditions can be used.

As a specific example of my method I may proceed as follows:—134 parts by weight of dehydrated nitrocellulose containing 34 parts by weight of ethyl alcohol and 20 100 parts by weight of nitrocellulose (40 parts soluble and 60 parts insoluble, say) are mixed with 50 parts of very finely pulverized potassium nitrate in a suitable mixer and colloided by the addition of about 66 25 parts by weight of ethyl ether (giving a ratio of ether to alcohol of about 2 to 1) with or without the use of brine refrigeration, the time of mixing being sufficient to insure a thorough distribution of the potassium nitrate throughout the colloid and from one to three hours usually sufficing, depending upon the efficiency of the mixer. The colloid after mixing is pressed into preliminary blocks by means of any suitable 30 press and the blocks are then pressed through dies having proper sized openings to give the desired diameter to the finished grains; the strings of powder are taken from the die to a granulating or cutting 35 machine and cut into grains of the desired length; from the cutting machine the grains are discharged into water, the temperature of the water being maintained under 65° C. and above the boiling point of ethyl ether, the water being preferably used in such 40 quantity that the boiling point of the solution is above 65° C. and the ethyl ether is retained in the solution; the treatment being continued for four days, more or less, until 45 substantially all salt and all solvent are both removed from the powder, the water being changed several times to render the extraction of the salts as complete as possible; after the removal of the salt and solvent 50 the powder is removed from the water, allowed to drain and then dried at a temperature of about 50° C. until the excess moisture is removed; the powder is then cooled, exposed to absorb moisture and graphited in the usual manner.

It will be understood that the systematic extraction of fresh portions of powder grains with the water which has been used for the extraction of a previous portion of powder grains can be arranged to take place

in such a way that a very strong solution can be obtained from which the nitrocellulose solvent can be recovered and the water evaporated and the salt recovered. Evidently, various modifications of proportions, 70 times, and temperatures, and so forth, may be made without departure from the spirit of my invention. Also, although I find highly desirable the use of a nitrocellulose mixture which is not wholly soluble in the 75 solvent used, and, also, prefer to use such a solvent for the nitrocellulose, and such a solid body, that both may be removed simultaneously, it will be understood that certain 80 features of advantage of the invention may be retained though either of these features be not used.

It will be seen that I have provided, in the art of increasing the porosity of dense nitrocellulose powder by incorporating a 85 soluble body in the nitrocellulose and ultimately dissolving out the body, a method whereby complications are avoided, a superior product produced, and the solid body and the solvent for the nitrocellulose conveniently removed from the product.

Having thus described my invention, what I claim as new is:—

1. The method of preparing nitrocellulose propellant powder which consists in colloid- 95 ing a mixture of nitrocellulose having a portion not soluble in, and a portion soluble in, the solvent used for colloid-ing, and incorporating a soluble solid body in the colloid, and then simultaneously, and in a single 100 step, removing said solvent and said solid body.

2. The method of preparing nitrocellulose propellant powder which consists in colloid- 105 ing, with a mixture of ethyl ether and ethyl alcohol, nitrocellulose less than 50% of which is soluble in said mixture, incorporating a metal nitrate in said nitrocellulose before the colloid-ing thereof is completed, forming the resulting composition into 110 grains, and then treating the latter with water to extract, simultaneously, and in a single step, the ether, alcohol, and metal nitrate.

3. The method of preparing porous die- 115 pressed nitrocellulose propellant powder which consists in colloid-ing with a solvent mixture of ethyl ether and ethyl alcohol, nitrocellulose less than 50% of which is soluble in said mixture, incorporating a water- 120 soluble solid body in the colloid, pressing the colloid through a die, cutting into grains the strings so formed, and then removing the solvent and solid body by treating with water.

4. The method of preparing nitrocellulose propellant powder which consists in colloid- 125 ing nitrocellulose with a solvent soluble in a given solvent, incorporating in the colloid a solid body soluble in the given solvent, and

then treating the colloid with the given solvent, and at a temperature below the boiling point of the resulting solution, thereby to simultaneously remove the nitrocellulose solvent and the solid body while retaining such solvent in said solution.

5. The method of preparing nitrocellulose propellant powder which consists in colloid-ing with a solvent soluble in a given solvent, 10 nitrocellulose less than 50% of which is soluble in the first named solvent, incorporating in the colloid a solid body soluble in the given solvent, and then treating the colloid with the given solvent, and at a temperature 15 below the boiling point of the resulting solution, thereby to simultaneously remove the nitrocellulose solvent and the solid body while retaining such solvent in said solution.

6. The method of preparing nitrocellulose 20 propellant powder which consists in colloid-ing nitrocellulose with a solvent mixture of ethyl ether and ethyl alcohol, incorporating a water soluble solid body in the colloid, and then treating the colloid with water, 25 and at a temperature below the boiling point of the resulting solution, thereby to simultaneously remove the solvent and solid body while retaining the solvent in the solution.

7. The method of preparing nitrocellulose 30 propellant powder which consists in colloid-ing with a solvent mixture of ethyl ether and ethyl alcohol, nitrocellulose less than 50% of which is soluble in said mixture, incorporating a water soluble solid body in 35 the colloid, and then treating the colloid

with water, and at a temperature below the boiling point of the resulting solution, thereby to simultaneously remove the solvent and solid body while retaining the solvent in the solution.

8. The method of preparing nitrocellulose propellant powder which consists in colloid-ing nitrocellulose with a solvent mixture of ethyl ether and ethyl alcohol, incorporating a water-soluble solid body in the colloid, 45 forming the resulting composition into desired shapes, and then treating the shapes with water above the boiling point of ethyl ether and below 65° C. and in such quantity as to give a solution of a boiling point above 50 65° C. to thereby simultaneously and in a single step substantially remove solvent and solid body from the powder.

9. The method of preparing nitrocellulose propellant powder which consists in colloid-ing with a solvent mixture of ethyl ether and ethyl alcohol, nitrocellulose less than 50% of which is soluble in said mixture, incorporating a water-soluble solid body in the colloid, forming the resulting composition 60 into desired shapes, and then treating the shapes with water above the boiling point of ethyl ether and below 65° C. and in such quantity as to give a solution of a boiling point above 65° C. to thereby simultaneously 65 and in a single step substantially remove solvent and solid body from the powder.

In testimony whereof I affix my signature.

WALTER PHILIP REGESTEIN.